



US011685871B2

(12) **United States Patent**  
**Galante-Fox et al.**

(10) **Patent No.:** **US 11,685,871 B2**  
(45) **Date of Patent:** **Jun. 27, 2023**

(54) **METHODS TO REDUCE FREQUENCY OF DIESEL PARTICULATE FILTER REGENERATION**

(71) Applicant: **Afton Chemical Corporation**, Richmond, VA (US)

(72) Inventors: **Julienne Galante-Fox**, Midlothian, VA (US); **Timothy J. Whalen**, Midlothian, VA (US); **Daniel Taylor**, Fredericksburg, VA (US)

(73) Assignee: **Afton Chemical Corporation**, Richmond, VA (US)

(\*) Notice: Subject to any disclaimer, the term of this patent is extended or adjusted under 35 U.S.C. 154(b) by 0 days.

(21) Appl. No.: **17/728,378**

(22) Filed: **Apr. 25, 2022**

(65) **Prior Publication Data**

US 2022/0325195 A1 Oct. 13, 2022

**Related U.S. Application Data**

(63) Continuation-in-part of application No. 16/930,815, filed on Jul. 16, 2020, now Pat. No. 11,312,915.

(60) Provisional application No. 62/876,115, filed on Jul. 19, 2019.

(51) **Int. Cl.**  
**C10L 1/222** (2006.01)

(52) **U.S. Cl.**  
CPC ..... **C10L 1/2222** (2013.01); **C10L 2230/22** (2013.01); **C10L 2270/026** (2013.01); **C10L 2290/12** (2013.01)

(58) **Field of Classification Search**

CPC ..... C10L 1/2222; C10L 2230/22; C10L

2270/026; C10L 2290/12; C10L 1/143; C10L 1/1985; C10L 1/1883; C10L 1/189; C10L 1/232; C10L 1/2383; C10L 2200/0446; C10L 10/06; C10L 10/18; C10L 10/02

See application file for complete search history.

(56)

**References Cited**

**U.S. PATENT DOCUMENTS**

|                |         |                                    |
|----------------|---------|------------------------------------|
| 3,015,668 A    | 1/1962  | Kozikowski                         |
| 4,152,499 A    | 5/1979  | Boerzel et al.                     |
| 4,234,435 A    | 11/1980 | Meinhardt et al.                   |
| 4,482,357 A    | 11/1984 | Hanlon                             |
| 5,266,223 A    | 11/1993 | Song et al.                        |
| 5,575,823 A    | 11/1996 | Wallace et al.                     |
| 6,056,792 A *  | 5/2000  | Barr ..... C10L 10/12<br>44/365    |
| 7,980,067 B2 * | 7/2011  | Barton ..... F01N 3/0253<br>60/299 |
| 8,529,643 B2   | 9/2013  | Galante-Fox et al.                 |
| 8,758,456 B2   | 6/2014  | Fang et al.                        |
| 8,852,297 B2   | 10/2014 | Fang et al.                        |

(Continued)

*Primary Examiner* — Pamela H Weiss

(74) *Attorney, Agent, or Firm* — Honigman LLP; Larry Zhang

(57)

**ABSTRACT**

The present disclosure relates to a method of reducing regeneration frequency of a diesel particulate filter in a vehicle combustsing diesel fuel. The method includes combusting a diesel fuel in a vehicle engine having a diesel particulate filter and wherein the diesel particulate filter requires regeneration thereof. The diesel fuel has less than about 50 ppmw of sulfur and one or more select additives to reduce a measured frequency of regeneration of the diesel particulate filter.

**19 Claims, 2 Drawing Sheets**



(56)

**References Cited**

U.S. PATENT DOCUMENTS

- 2003/0182848 A1\* 10/2003 Collier ..... C07C 51/414  
44/365  
2006/0080954 A1\* 4/2006 Bardasz ..... C10M 159/20  
60/297  
2010/0011748 A1\* 1/2010 Yokota ..... F01N 3/106  
60/311  
2010/0043408 A1\* 2/2010 Girot ..... F02D 41/029  
60/287  
2013/0333650 A1 12/2013 Fang et al.

\* cited by examiner



FIG. 1



FIG. 2

## METHODS TO REDUCE FREQUENCY OF DIESEL PARTICULATE FILTER REGENERATION

### CROSS-REFERENCE TO RELATED APPLICATIONS

This application is a continuation-in-part of U.S. patent application Ser. No. 16/930,815, filed Jul. 16, 2020, which claims priority to U.S. Provisional Application No. 62/876,115, filed Jul. 19, 2019, which are both incorporated herein by reference.

### TECHNICAL FIELD

The present disclosure relates to methods for reducing regeneration frequency of a diesel particulate filter in a vehicle combusting diesel fuel, and more particularly, to the use of one or more diesel performance additives to reduce measured regeneration frequency and improve fuel economy.

### BACKGROUND

Diesel engines commonly result in combustion contaminants and particulates that tend to be undesired for a variety of reasons. The contaminants and particulates are often due to the incomplete combustion that tends to be inherent in the diesel engine and often results in small soot particles. A diesel particulate filter or DPF is a filtration device employed on modern vehicles combusting diesel fuel to remove the particulate and soot from the exhaust gas stream of the diesel engine.

During normal use, the DPF accumulates soot and particulate on or in the filter media. The filter can either be replaced or, more commonly, regenerated to burn off the accumulated soot. Regeneration is often achieved by increasing exhaust gas temperatures either through passive or active means in conjunction with injecting excess fuel into the cylinders. Such extra injections of fuel can lead to reductions in fuel economy.

### BRIEF DESCRIPTION OF THE FIGURES

FIG. 1 is a graph of regeneration frequency comparing the frequency of regeneration of a baseline or unadditized fuel to an additized diesel fuel.

FIG. 2 is a graph of DPF backpressure of a baseline or unadditized fuel to an additized diesel fuel.

### SUMMARY

In some aspects or embodiments of the present disclosure, a method of reducing measured regeneration frequency of a diesel particulate filter in a vehicle combusting diesel fuel is provided. In one approach, the method comprises (a) combusting a diesel fuel in a vehicle engine, wherein the vehicle includes a diesel particulate filter associated with the engine and wherein the diesel particulate filter requires regeneration thereof. The diesel fuel has less than about 50 ppmw of sulfur and one or more additives selected from (i) a hydrocarbyl substituted dicarboxylic anhydride derivative prepared by reacting a hydrocarbyl-substituted succinic acylating agent with an amine, polyamine, or alkyl amine having one or more primary, secondary, or tertiary amino groups; (ii) a quaternary ammonium internal salt obtained from amines or polyamines that is substantially devoid of any free

anion species; (iii) hydrocarbyl-substituted quaternary ammonium cationic salt formed by reacting an alkylating or quaternizing agent with a wide variety of hydrocarbyl-substituted tertiary amine compounds; (iv) a reaction product of a hydrocarbyl carbonyl compound and an amine compound selected from the group consisting of guanidine, urea, thiourea, and combinations thereof, and/or (v) alkoxylated phenol resins. Next, the method includes (b) regenerating the diesel particulate filter while combusting the diesel fuel; and (c) comparing the frequency of regeneration of the diesel particulate filter when combusting the diesel fuel comprising the one or more additives with the frequency of regeneration of the diesel particulate filter when combusting a diesel fuel which is devoid of the one or more additives; wherein the frequency of regenerations per 1000 miles of the diesel particulate filter when combusting the diesel fuel comprising the one or more additives is lower than a frequency of regenerations per 1000 miles of the diesel particulate filter when combusting a diesel fuel in the engine devoid of the one or more additives.

In other aspects or embodiments, the method of the previous paragraph may be combined with one or more optional features or method steps in any combination or sub-combination thereof. These other embodiments or sub-embodiments include one or more of the following: wherein the quaternary ammonium cationic salt additive has the structure of Formula VII:



wherein each X is a bivalent moiety selected from the group consisting of  $-\text{O}-$ ,  $-\text{N}(R_{20})-$ ,  $-\text{C}(\text{O})-$ ,  $-\text{C}(\text{O})\text{O}-$ , or  $-\text{C}(\text{O})\text{NR}_{20}$ ; each  $R_{15}$ ,  $R_{16}$ , and  $R_{17}$  are independently alkyl groups containing 1 to 8 carbon atoms;  $R_{18}$  and  $R_{19}$  are independently selected from an alkyl group, acyl group, or a hydrocarbyl substituted acyl group, the hydrocarbyl substituent of one or both of  $R_{18}$  and  $R_{19}$  having a number average molecular weight of about 700 or greater;  $R_{20}$  is independently a hydrogen or a group selected from  $\text{C}_{1-6}$  aliphatic, phenyl, or alkylphenyl; each m is independently an integer of 0 or 1 with at least one m being 1; each n is independently an integer of 1 to 10; and  $M^\ominus$  is a carboxylate; and/or wherein the carboxylate of Formula VII is oxalate, salicylate, or combinations thereof, and/or wherein X of Formula VII is  $-\text{O}-$  or  $-\text{NH}-$ ; and/or wherein the amine used to form the quaternary ammonium cationic salt additive has the structure of Formula VIII:



wherein each X is a bivalent moiety selected from the group consisting of  $-\text{O}-$ ,  $-\text{N}(R_{20})-$ ,  $-\text{C}(\text{O})-$ ,  $-\text{C}(\text{O})\text{O}-$ , or  $-\text{C}(\text{O})\text{NR}_{20}$ ; each  $R_{15}$  and  $R_{16}$  are independently alkyl groups containing 1 to 8 carbon atoms; each m is independently an integer of 0 or 1 with at least one m being 1; each n is independently an integer of 1 to 10; and/or wherein X is an oxygen atom or nitrogen atom; and/or wherein X is preferably an oxygen atom; and/or wherein the quaternary ammonium cationic salt additive of Formula VII is derived from 3-(2-(dimethylamino)ethoxy)propylamine, N,N-dimethyl dipropyletriamine, or mixtures thereof, and/or wherein  $R_{18}$  and  $R_{19}$  of Formula VII, together with the nitrogen atom to which they are attached, combine to form a hydrocarbyl substituted succinimide; and/or wherein the hydrocarbyl substituent has a number average molecular weight of about 700 to about 2,500; and/or wherein X is an oxygen atom and wherein  $R_{19}$  and  $R_{19}$  of Formula VI,

together with the nitrogen atom to which they are attached, combine to form a hydrocarbyl substituted succinimide with the hydrocarbyl substituent having a number average molecular weight of about 700 to about 1,500 as measured by GPC using polystyrene as a calibration reference; and/or wherein M is derived from dimethyl oxalate, methyl salicylate, or combinations thereof; and/or wherein the alkoxylated phenol polymer (v) has the general structure of Formula XII:  $(R_{28})_p-PH-(CH_2)_m-C(O)O-(AO)_n-R_{29}$  (Formula XII) wherein PH is a phenyl group optionally substituted with  $R_{28}$  groups where each  $R_{28}$  is independently a C1 to C4 alkyl or alkoxy group;  $R_{29}$  is a C1 to C10 linear or branched alkyl group; AO is an alkylene oxide derived group; and/or wherein n is an integer that may range from 1 to 100; m may be an integer of 1 or 2; and p is an integer of 0, 1 or 2; and wherein  $R_{28}$  and/or  $R_{29}$  is a branched alkyl group selected from iso-propyl (prop-2-yl), sec-butyl (but-2-yl), iso-butyl (2-methyl-prop-1-yl) and/or tert-butyl group, or a 2-ethyl hexyl group, or combinations thereof; and/or wherein the diesel fuel includes about 5 ppmw to about 150 ppmw of additive (iii) and about 1 ppmw to about 35 ppmw of additive (v).

In yet other approaches and embodiments, the methods may also include wherein the diesel fuel includes less than about 20 weight percent of bio-generated diesel fuel additives selected from the group consisting of fatty acid methyl esters, hydrotreated vegetable oil, soybean methyl esters, palm methyl esters, and combinations thereof, and/or wherein the regeneration occurs when the engine injects excess diesel fuel into a cylinder to increase the exhaust gas temperature to exceed a predetermined temperature and reacts with a catalyst (DOC) causing an elevated temperature across the catalyst and into the diesel particulate filter; and/or wherein the elevated temperature oxidizes soot trapped in or on the diesel particulate filter and regenerates or cleans the filter; and/or wherein the regeneration is measured when the exhaust gas stream exceeds about 480° C.; and/or wherein the reduction in regeneration frequency occurs immediately upon combusting the diesel fuel having the one or more additives; and/or wherein the regeneration frequency per 1000 miles is about 0.5 to about 20 percent lower than the regeneration frequency per 1000 miles of a diesel fuel without the one or more additives; and/or wherein diesel fuel further include additives selected from thiazole, triazole, thiadiazole, and combinations thereof; and/or wherein the thiazole, triazole, thiadiazole are selected from benzotriazole, tolyltriazole, octyltriazole, decyltriazole, dodecyltriazole, 2-mercapto benzothiazole, 2,5-dimercapto-1,3,4-thiadiazole, 2-mercapto-5-hydrocarbylthio-1,3,4-thiadiazoles, 2-mercapto-5-hydrocarbyldithio-1,3,4-thiadiazoles, 2,5-bis(hydrocarbylthio)-1,3,4-thiadiazoles, and 2,5-bis(hydrocarbyldithio)-1,3,4-thiadiazoles, and combinations thereof.

#### DETAILED DESCRIPTION

The present disclosure relates to methods of combusting a diesel fuel and measuring a regeneration frequency of a diesel particulate filter (DPF) in a vehicle combusting diesel fuel to provide a reduction in measured DPF regeneration frequency. As explained in the background, most diesel engines employ the DPF to remove soot and other combustion particulates from the exhaust gas. These filters are associated with diesel engines and commonly located downstream of the engine in the exhaust systems. They may be found after a turbocharger or positioned before or after a catalytic converter in the exhaust system. These filters need

regeneration from time to time and commonly employ one or more regeneration techniques to renew the filter. Regeneration of the DPF occurs when the exhaust temperature is high enough to react with or activate a diesel oxidation catalyst (DOC) to burn off the accumulated soot and particulate on the filter upon injecting excess diesel fuel into the engine. Regeneration commonly involves either an active regeneration cycle or a passive regeneration cycle. An active regeneration occurs when the exhaust gas and catalyst temperature is not high enough to light off the DOC. In this instance, the vehicle ECU adjusts engine parameters (such as, but not limited to, injection timing, turbo geometry, etc.) to increase exhaust temperature while also injecting the excess fuel into the cylinder to cause an exothermic reaction which then oxidizes the soot in the DPF and cleans or “regenerates” the filter. Likewise, a passive regeneration is when the engine exhaust temperature is already high enough to facilitate the reaction of excess fuel in the DOC and the ECU only needs to inject excess fuel for the regeneration to occur. This later situation usually happens at high RPM or high load conditions.

The regeneration cycles tend to substantially increase fuel consumption, and thus, decrease fuel economy of the vehicle. Discovered herein, on the other hand, are methods of combusting diesel fuel and regenerating the DPF by reducing the frequency of measured regenerations and, thus, the overall fuel consumption of the diesel engine at the same time.

In one aspect, the methods herein include combusting a diesel fuel in a vehicle engine, wherein the vehicle includes a diesel particulate filter associated with the engine and the frequency of measured regeneration is decreased by combusting a diesel fuel having a select combination of additives that surprisingly decrease the measured regeneration frequency. In one approach, the method includes combusting diesel fuel having less than about 50 ppmw of sulfur (that is, low sulfur diesel fuel or, in other approaches, ultra-low sulfur diesel fuel having less than 15 ppmw of sulfur) and one or more additives selected from (i) a hydrocarbyl substituted dicarboxylic anhydride derivative prepared by reacting a hydrocarbyl-substituted succinic acylating agent with an amine, polyamine, or alkyl amine having one or more primary, secondary, or tertiary amino groups; (ii) a quaternary ammonium internal salt obtained from amines or polyamines that is substantially devoid of any free anion species; (iii) hydrocarbyl-substituted quaternary ammonium cationic salts formed by reacting an alkylating or quaternizing agent with a wide variety of hydrocarbyl-substituted tertiary amine compounds; (iv) a reaction product of a hydrocarbyl carbonyl compound and an amine compound selected from the group consisting of guanidine, urea, thiourea, and combinations thereof, and/or (v) alkoxyLATED phenol or phenol formaldehyde resin additives. In other approaches, the methods include combusting the low sulfur diesel fuel with various combinations of additives (i) to (v) or, in other approaches, select individual additives of (i) to (v).

The methods may further include regenerating the diesel particulate filter, typically using an active regeneration, a passive regeneration, other suitable regeneration cycle, while combusting the diesel fuel (which may also include an excess fuel injection) and measuring a frequency of regenerations of the diesel particulate filter. When combusting the diesel fuel and the select additive compositions herein, the measured frequency of regenerations per 1000 miles is lower than the measured frequency of regenerations per 1000 miles of the diesel particulate filter when combusting a

diesel fuel in the engine without or devoid of the one or more additives. As used herein, an excess fuel injection generally means additional diesel fuel beyond the stoichiometric amount required for combustion to normally operate the diesel engine. As used herein, without or devoid of generally mean no active amounts, such as less than about 5 ppm of active additives, less than about 1 ppm, and preferably no active DPF additives. The excess fuel is vaporized and mixed with the exhaust gases.

In some approaches or embodiments, the DPF regeneration reduction additives may be any combination of additives (i) to (v) or any one additive (i) to (v) present in the diesel fuel in amounts (as a combination or individual additive) from about 10 ppmw to about 150 ppmw. In other embodiments, an individual additive or combination of total active DPF regeneration reduction additives may be present in the diesel fuel at least about 10 ppmw, at least about 20 ppmw, at least about 40 ppmw, at least about 50 ppmw, at least about 60 ppmw, at least about 80 ppmw, or at least about 100 ppmw and less than about 150 ppm, less than about 140 ppmw, less than about 130 ppmw, less than about 120 ppmw, less than about 110 ppmw, less than about 100 ppmw, less than about 90 ppmw, less than about 80 ppmw, or less than about 70 ppmw where ppmw is parts per million by weight. Weights may also be measured by volume as needed for a particular application.

In other approaches or embodiments, the diesel fuel may include about 5 ppmw to about 150 ppmw of additive (i) and about 5 ppmw to about 50 ppmw of additive (ii) at the same time. In yet other approaches or other embodiments, the diesel fuel includes about 35 ppmw to about 150 ppmw of the additive (i) and about 5 ppmw to about 50 ppmw of additive (iv) at the same time. In additional embodiments, the diesel fuel may include about 5 ppmw to about 100 ppmw of additive (i) and about 1 ppmw to about 35 ppmw of additive (ii). In still other embodiments, the diesel fuel includes about 35 ppmw to about 150 ppmw of the additive (i) and about 5 ppmw to about 50 ppmw of additive (iv). In still other embodiments, the diesel fuel may include about 1 to about 60 ppmv of additive (iii) or, alternatively, about 1 to about 200 ppmv of additive (iii) and 1 to about 50 ppmw of additive (v). Weights may be in volume or by mass depending on the application. Other ranges and combinations of additives within the noted endpoints may also be contemplated by this disclosure. As used throughout this disclosure and unless stated otherwise, the amount of the DPF additives are noted in active amounts and does not include amounts of solvents or other carriers.

In some embodiments, the one or more additives selected may include the hydrocarbyl substituted dicarboxylic anhydride derivative alone, a quaternary ammonium internal salt alone; a quaternary ammonium cationic salt alone, the reaction product of the hydrocarbyl carbonyl compound and the amine compound alone, or the alkoxylated phenol or phenol formaldehyde polymer alone. In other embodiments, the one or more additives selected may comprise various combination of additives including (i) one or more of the hydrocarbyl substituted dicarboxylic anhydride derivative, (ii) the quaternary ammonium internal salt, (iii) the quaternary ammonium cationic salt, (iv) the reaction product of the hydrocarbyl carbonyl compound and the amine compound; and/or (v) the alkoxylated phenol formaldehyde resin. In still other embodiments, the one or more additives selected may include a combination of two or more additives including, for instance, (a) the hydrocarbyl substituted dicarboxylic anhydride derivative and the quaternary ammonium internal salt, (b) the hydrocarbyl substituted dicarboxylic

anhydride derivative and the reaction product of the hydrocarbyl carbonyl compound and the amine compound, (c) the quaternary ammonium internal salt and the reaction product of the hydrocarbyl carbonyl compound and the amine compound, or (d) the quaternary ammonium cationic salt and the alkoxylated phenol polymer or phenol formaldehyde polymer. Each of these additives suitable for the methods herein are described in more detail below.

#### Hydrocarbyl Substituted Dicarboxylic Anhydride Derivative

One of the discovered additives to reduce measured DPF regeneration frequency when combusting diesel fuel is a hydrocarbyl substituted dicarboxylic anhydride derivative. In one approach, this additive may be prepared by reacting a hydrocarbyl-substituted succinic acylating agent with an amine, polyamine, or alkyl amine having one or more primary, secondary, or tertiary amino groups. In some embodiments, the hydrocarbyl substituted dicarboxylic anhydride derivative includes hydrocarbyl succinimides, succinamides, succinimide-amides and succinimide-esters. These nitrogen-containing derivatives of hydrocarbyl succinic acylating agents may be prepared by reacting a hydrocarbyl-substituted succinic acylating agent with an amine, polyamine, or alkyl amine having one or more primary, secondary, or tertiary amino groups.

In some approaches or embodiments, the hydrocarbyl substituted dicarboxylic anhydride derivative may include a hydrocarbyl substituent having a number average molecular weight ranging from about 450 to about 3000 as measured by GPC using polystyrene as reference. The derivative may be selected from a diamide, acid/amide, acid/ester, diacid, amide/ester, diester, and imide. Such derivative may be made from reacting a hydrocarbyl substituted dicarboxylic anhydride with ammonia, a polyamine, or an alkyl amine having one or more primary, secondary, or tertiary amino groups. In some embodiments, the polyamine or alkyl amine may be tetraethylene pentamine (TEPA), triethylenetetramine (TETA), and the like amines. In other approaches, the polyamine or alkyl amine may have the formula  $H_2N—((CH_2)_q—NH)_r—H$ , wherein  $R_1$  is hydrogen or an alkyl group having from 1 to 4 carbon atoms,  $q$  is an integer of from 1 to 4 and  $r$  is an integer of from 1 to 6, and mixtures thereof. In other approaches, a molar ratio of the hydrocarbyl substituted dicarboxylic anhydride reacted with the ammonia, polyamine, or alkyl amine may be from about 0.5:1 to about 2:1, in other approaches about 1:1 to about 2:1.

In other approaches, the hydrocarbyl substituted dicarboxylic anhydride may be a hydrocarbyl carbonyl compound of the Formula I:

(Formula I)



where  $R_2$  is a hydrocarbyl group derived from a polyolefin. In some aspects, the hydrocarbyl carbonyl compound may be a polyalkylene succinic anhydride reactant wherein  $R_2$  is a hydrocarbyl moiety, such as for example, a polyalkenyl radical having a number average molecular weight of from about 450 to about 3000 as measured by GPC using poly-

styrene as reference. For example, the number average molecular weight of  $R_2$  may range from about 600 to about 2500, or from about 700 to about 1500, as measured by GPC using polystyrene as reference. A particularly useful  $R_2$  has a number average molecular weight of about 950 to about 1000 Daltons (as measured by GPC using polystyrene as reference) and comprises polyisobutylene. Unless indicated otherwise, molecular weights in the present specification are number average molecular weights as measured by GPC using polystyrene as reference.

The  $R_2$  hydrocarbyl moiety may include one or more polymer units chosen from linear or branched alkenyl units. In some aspects, the alkenyl units may have from about 2 to about 10 carbon atoms. For example, the polyalkenyl radical may comprise one or more linear or branched polymer units chosen from ethylene radicals, propylene radicals, butylene radicals, pentene radicals, hexene radicals, octene radicals and decene radicals. In some aspects, the  $R_2$  polyalkenyl radical may be in the form of, for example, a homopolymer, copolymer or terpolymer. In one aspect, the polyalkenyl radical is isobutylene. For example, the polyalkenyl radical may be a homopolymer of polyisobutylene comprising from about 10 to about 60 isobutylene groups, such as from about 20 to about 30 isobutylene groups. The polyalkenyl compounds used to form the  $R_2$  polyalkenyl radicals may be formed by any suitable methods, such as by conventional catalytic oligomerization of alkenes.

In some aspects, high reactivity polyisobutenes having relatively high proportions of polymer molecules with a terminal vinylidene group may be used to form the  $R_2$  group. In one example, at least about 60%, such as about 70% to about 90%, of the polyisobutenes comprise terminal olefinic double bonds. High reactivity polyisobutenes are disclosed, for example, in U.S. Pat. No. 4,152,499, the disclosure of which is herein incorporated by reference in its entirety.

In some aspects, approximately one mole of maleic anhydride may be reacted per mole of polyalkylene, such that the resulting polyalkenyl succinic anhydride has about 0.8 to about 1 succinic anhydride group per polyalkylene substituent. In other aspects, the molar ratio of succinic anhydride groups to polyalkylene groups may range from about 0.5 to about 3.5, such as from about 1 to about 1.1.

The hydrocarbyl carbonyl compounds may be made using any suitable method. One example of a method for forming a hydrocarbyl carbonyl compound comprises blending a polyolefin and maleic anhydride. The polyolefin and maleic anhydride reactants are heated to temperatures of, for example, about 150° C. to about 250° C., optionally, with the use of a catalyst, such as chlorine or peroxide. Another exemplary method of making the polyalkylene succinic anhydrides is described in U.S. Pat. No. 4,234,435, which is incorporated herein by reference in its entirety.

In the hydrocarbyl substituted dicarboxylic anhydride derivative, the polyamine reactant may be an alkylene polyamine. For example, the polyamine may be selected from ethylene polyamine, propylene polyamine, butylenes polyamines, and the like. In one approach, the polyamine is an ethylene polyamine that may be selected from ethylene diamine, diethylene triamine, triethylene tetramine, tetraethylene pentamine, pentaethylene hexamine, and N, N'-(imino-di-2,1,ethanediyl) bis-1,3-propanediamine. A particularly useful ethylene polyamine is a compound of the formula  $H_2N-((CHR_1-(CH_2)_q NH)_r-H$ , wherein  $R_1$  is hydrogen,  $q$  is 1 and  $r$  is 1.

In yet further approaches, the hydrocarbyl substituted dicarboxylic anhydride derivative is a compound of Formula II



(Formula II)

wherein  $R_4$  is a hydrocarbyl group (such as polyisobutylene and/or the other above described  $R_2$  moieties) and  $R_5$  is a hydrogen, an alkyl group, an aryl group, —OH, —NHR<sub>6</sub>, or a polyamine, or an alkyl group containing one or more primary, secondary, or tertiary amino groups. In some approaches,  $R_5$  is derived from ethylene diamine, diethylene triamine, triethylene tetraamine, tetraethylene pentamine, pentaethylene hexamine, N,N'-(imino-di-2,1,ethanediyl) bis-1,3-propanediamine and combinations thereof. In some embodiments,  $R_4$  is a hydrocarbyl group and  $R_5$  is hydrogen, an alkyl group, an aryl group, —OH, —NHR<sub>5</sub>, or a polyamine and wherein R5' is a hydrogen or an alkyl group. In other embodiments, the additive of Formula II includes a hydrocarbyl substituted succinimide derived from ethylene diamine, diethylene triamine, triethylene tetraamine, tetraethylene pentamine, pentaethylene hexamine, N,N'-(imino-di-2,1,ethanediyl) bis-1,3-propanediamine and combinations thereof. In still other embodiments,  $R_4$  in the compound of Formula I is a hydrocarbyl group having a number average molecular weight from about 450 to about 3,000 and  $R_5$  is derived from tetraethylene pentamine and derivatives thereof.

In yet other approaches  $R_5$  is a compound of Formula III:



(Formula III)

wherein A is NR<sub>6</sub> or an oxygen atom, R<sub>6</sub>, R<sub>7</sub>, and R<sub>8</sub> are independently a hydrogen atom or an alkyl group, m and p are integers from 2 to 8; and n is an integer from 0 to 4. In some approaches, R<sub>7</sub> and R<sub>6</sub> of Formula III, together with the nitrogen atom to which they are attached, form a 5 membered ring.

In yet other approaches, the diesel fuel herein includes about 5 to about 150 ppmw of the active hydrocarbyl substituted dicarboxylic anhydride derivative (i), in other approaches, about 5 to about 100 ppmw, or about 30 to about 150 ppmw, or about 30 to about 120 ppmw, or about 5 to about 90 ppmw, and in yet other approaches, 5 to 50 ppmw. In yet other approaches, the diesel fuel herein includes an amount of this additive ranging from at least about 5 ppmw, at least about 10 ppmw, at least about 20 ppmw, at least about 30 ppmw, or at least about 40 to less than about 150 ppmw, less than about 120 ppmw, less than about 100 ppmw, less than about 90 ppmw, less than about 80 ppmw, less than about 70 ppmw, less than about 50 ppm, less than about 40 ppm, or less than about 30 ppmw. In some approaches, when then PIBSA to amine ratio is about 0.5:1 to about 1.2:1, then the diesel fuel includes about 35 to about 150 ppmw of this additive. In other approaches, when the PIBSA to amine ratio is about 1.4:1 to about 2.0:1, then the diesel fuel includes about 5 to about 100 ppmw of the additive.

A diesel fuel additive or concentrate including this compound may have about 10 to about 80 weight percent of active additive.

## Quaternary Ammonium Internal Salt

Another possible additive in the blend to reduce measured DPF regeneration frequency when combusting diesel fuel is a quaternary ammonium internal salt. In some embodiments, the quaternary ammonium internal salt may be obtained from amines or polyamines that are substantially devoid of any free anion species. For example, such additive may be made by reacting a tertiary amine of Formula IV:



(Formula IV)

wherein each of R<sub>9</sub>, R<sub>10</sub>, and R<sub>11</sub> is selected from hydrocarbyl groups containing from 1 to 200 carbon atoms, with a halogen substituted C2-C8 carboxylic acid, ester, amide, or salt thereof. What is generally to be avoided in the reaction is quaternizing agents selected from the group consisting of hydrocarbyl substituted carboxylates, carbonates, cyclic-carbonates, phenates, epoxides, or mixtures thereof. In one embodiment, the halogen substituted C2-C8 carboxylic acid, ester, amide, or salt thereof may be selected from chloro-, bromo-, fluoro-, and iodo-C2-C8 carboxylic acids, esters, amides, and salts thereof. The salts may be alkali or alkaline earth metal salts selected from sodium, potassium, lithium calcium, and magnesium salts. A particularly useful halogen substituted compound for use in the reaction is the sodium or potassium salt of a chloroacetic acid.

As used herein the term "substantially devoid of free anion species" means that the anions, for the most part are covalently bound to the product such that the reaction product as made does not contain any substantial amounts of free anions or anions that are ionically bound to the product. In one embodiment, "substantially devoid" means from 0 to less than about 2 wt. % of free anion species or any range therein.

In another approach or embodiment, a tertiary amine including monoamines and polyamines may be reacted with the halogen substituted acetic acid or derivative thereof to provide the first detergent additive of the synergistic mixture. Suitable tertiary amine compounds are those of Formula V:



(Formula V)

where each of R<sub>9</sub>, R<sub>10</sub>, and R<sub>11</sub> is selected, as noted above, from hydrocarbyl groups containing from 1 to 200 carbon atoms. Each hydrocarbyl group R<sub>9</sub> to R<sub>11</sub> may independently be linear, branched, substituted, cyclic, saturated, unsaturated, or contain one or more hetero atoms. Suitable hydrocarbyl groups may include, but are not limited to alkyl groups, aryl groups, alkylaryl groups, arylalkyl groups, alkoxy groups, aryloxy groups, amido groups, ester groups, imido groups, and the like. Any of the foregoing hydrocarbyl groups may also contain hetero atoms, such as oxygen or nitrogen atoms. Particularly suitable hydrocarbyl groups may be linear or branched alkyl groups. Some representative examples of amine reactants which can be reacted to yield compounds of this disclosure include, but are not limited to, trimethyl amine, triethyl amine, tri-n-propyl amine, dim-

ethylethyl amine, dimethyl lauryl amine, dimethyl oleyl amine, dimethyl stearyl amine, dimethyl eicosyl amine, dimethyl octadecyl amine, N-methyl piperidine, N,N'-dimethyl piperazine, N-methyl-N-ethyl piperazine, N-methyl morpholine, N-ethyl morpholine, N-hydroxyethyl morpholine, pyridine, triethanol amine, triisopropanol amine, methyl diethanol amine, dimethyl ethanol amine, lauryl diisopropanol amine, stearyl diethanol amine, dioleyl ethanol amine, dimethyl isobutanol amine, methyl diisooctanol amine, dimethyl propenyl amine, dimethyl butenyl amine, dimethyl octenyl amine, ethyl didodecenyl amine, dibutyl eicosenyl amine, triethylene diamine, hexa-methylenetetramine, N,N,N',N'-tetramethylmethylethylenediamine, N,N,N',N'-tetramethyl-propylenediamine, N,N,N',N'-tetraethyl-1,3-propanediamine, methyldi-cyclohexyl amine, 2,6-dimethylpyridine, dimethylcyclohexylamine, C10-C30-alkyl or alkenyl-substituted amidopropyldimethylamine, C12-C200-alkyl or alkenyl-substituted succinic-carbonyl-dimethylamine, and the like. A suitable first cleaning additive may be the internal salts of oleyl amidopropyl dimethyl-amino or oleyl dimethyl amine.

If the amine contains solely primary or secondary amino groups, it may be necessary to alkylate at least one of the primary or secondary amino groups to a tertiary amino group prior to the reaction with the halogen substituted C2-C8 carboxylic acid, ester, amide, or salt thereof. In one embodiment, alkylation of primary amines and secondary amines or mixtures with tertiary amines may be exhaustively or partially alkylated to a tertiary amine. It may also be necessary to properly account for the hydrogens on the nitrogen and provide base or acid as required (e.g., alkylation up to the tertiary amine requires removal (neutralization) of the hydrogen (proton) from the product of the alkylation). If alkylating agents, such as, alkyl halides or dialkyl sulfates are used, the product of alkylation of a primary or secondary amine is a protonated salt and needs a source of base to free the amine for further reaction.

The halogen substituted C2-C8 carboxylic acid, ester, amide, or salt thereof for use in making the first cleaning additive may be derived from a mono-, di-, or tri-chlorobromo-, fluoro-, or iodo-carboxylic acid, ester, amide, or salt thereof selected from the group consisting of halogen-substituted acetic acid, propanoic acid, butanoic acid, isopropanoic acid, isobutanoic acid, tert-butanoic acid, pentanoic acid, heptanoic acid, octanoic acid, halo-methyl benzoic acid, and isomers, esters, amides, and salts thereof. The salts of the carboxylic acids may include the alkali or alkaline earth metal salts, or ammonium salts including, but not limited to the Na, Li, K, Ca, Mg, triethyl ammonium and triethanol ammonium salts of the halogen-substituted carboxylic acids. A particularly suitable halogen substituted carboxylic acid, or salt thereof may be selected from chloroacetic acid and sodium or potassium chloroacetate. The amount of halogen substituted C2-C8 carboxylic acid, ester, amide, or salt thereof relative to the amount of tertiary amine reactant may range from a molar ratio of about 1:0.1 to about 0.1:1.0.

The internal salts made according to the foregoing procedure may include, but are not limited to (1) hydrocarbyl substituted compounds of the formula R"—NMe<sub>2</sub>CH<sub>2</sub>COO where R" is from C1 to C30 or a substituted amido group; (2) fatty amide substituted internal salts; and (3) hydrocarbyl substituted imide, amide, or ester internal salts wherein the hydrocarbyl group has 8 to 40 carbon atoms. Particularly suitable internal salts may be selected from the group consisting of polyisobutetyl substituted succinimide, succinic diamide, and succinic diester internal salts; C8-C40

## 11

alkenyl substituted succinimide, succinic diamide, and succinic diester internal salts; oleyl amidopropyl dimethylamino internal salts; and oleyl dimethylamino internal salts.

In yet another approach or embodiment, the quaternary ammonium internal salt may be a quaternary ammonium internal salt of Formula VI:



(Formula VI)

wherein Rand R' are independently alkylene linkers having 1 to 10 carbon atoms (in other approaches 1 to 3 carbon atoms); R<sub>12</sub> is independently a hydrocarbyl group or optionally substituted hydrocarbyl group, or an aryl group or optionally substituted aryl group; R<sub>13</sub> is independently a linear or branched C1 to C4 alkyl group; R<sub>14</sub> is a hydrogen atom or a C1 to C4 alkyl group. The internal salts of Formula I may also be substantially devoid of free anion species as discussed above. In some embodiments, R and R' are independently alkylene linkers having 1 to 10 carbon atoms; R<sub>12</sub> is a hydrocarbyl group or optionally substituted hydrocarbyl group, or an aryl group or optionally substituted aryl group; R<sub>13</sub> is independently a linear or branched C1 to C4 alkyl group; and R<sub>14</sub> is hydrogen or a C1 to C4 alkyl group. In other embodiments, R and R' are independently alkylene linkers having 1 to 3 carbon atoms and R<sub>12</sub> is a C8 to C20 hydrocarbyl group.

In another approach, the quaternary ammonium internal salt may include the compound of Formula VI above wherein R is a propylene linker, R is a methylene linker, R<sub>12</sub> is a C8 to C20 hydrocarbyl group, and R<sub>13</sub> is a methyl group. In some embodiments, R<sub>12</sub> is derived from an oleyl fatty acid. In yet other approaches, the additive is selected from oleyl amidopropyl dimethylamine internal salts or oleyl dimethylamino internal salts. In some approaches, such additive may be substantially devoid of free anion species.

In some approaches, the diesel fuel herein may include about 1 to about 35 ppmw of this additive (ii), and in other approaches, about 5 to about 25 ppmw, and in yet other approaches, about 5 to about 20 ppmw. In yet other approaches, the diesel fuel may include an amount of this additive ranging from at least about 1 ppmw, at least about 5 ppmw, or at least about 10 ppmw to less than about 30 ppmw, less than about 25 ppmw, less than about 20 ppmw, less than about 15 ppmw, or less than about 10 ppmw.

In yet further approaches, a diesel fuel additive or concentrate may include, on an active basis, about 2 to about 20 weight percent of this compound.

## Quaternary Ammonium Cationic Salt

Another possible additive in the blend to reduce measured DPF regeneration frequency when combusting diesel fuel is a quaternary ammonium cationic salt. In approaches, the quaternary ammonium cationic salt herein includes a quaternary ammonium salt formed through a reaction between an alkyl carboxylate and an amide or imide compound obtained by reacting a hydrocarbyl substituted acylating agent, such as a high molecular weight hydrocarbyl substituted acylating agent, and an amine.

In one approach, suitable quaternary ammonium cationic salts have the structure of Formula VII



wherein each X is a bivalent moiety selected from the group consisting of —O—, —N(R<sub>20</sub>)—, —C(O)—, —C(O)O—, or —C(O)NR<sub>20</sub>; each R<sub>15</sub>, R<sub>16</sub>, and R<sub>17</sub> are independently alkyl groups containing 1 to 8 carbon atoms; R<sub>18</sub> and R<sub>19</sub> are independently selected from an alkyl group, an acyl group, or a hydrocarbyl substituted acyl group and, optionally, R<sub>18</sub> and R<sub>19</sub> together with the N atom to which they are attached, combine to form a ring moiety (such as a succinimide), the hydrocarbyl substituent of one or both of R<sub>18</sub> and R<sub>19</sub> having a number average molecular weight of about 700 or greater (as described herein); R<sub>20</sub> is independently a hydrogen or a group selected from C<sub>1-6</sub> aliphatic, phenyl, or alkylphenyl; each m is independently an integer of 0 or 1 with at least one m being 1; each n is independently an integer of 1 to 10; and M<sup>⊖</sup> is a carboxylate.

In one approach of this aspect, the amine used to form the quaternary ammonium cationic salt additive may have the structure of Formula VIII



(Formula VIII)

with X, R<sub>15</sub>, R<sub>16</sub> and integers n and m as defined above. In a preferred approach, the X moiety is an oxygen atom or nitrogen atom, and more preferably, an oxygen atom. In a preferred approach, the amine used for the quaternary ammonium cationic salt is 3-(2-(dimethyl amino)ethoxy) propylamine; N,N-dimethyldipropylenetriamine, or mixtures thereof.

Any of the foregoing described tertiary amines may be reacted with a hydrocarbyl substituted acylating agent having the noted high molecular weight hydrocarbyl substituent described herein to form the second quaternary ammonium salt additive. In approaches, the hydrocarbyl substituted acylating agent may be selected from a hydrocarbyl substituted mono- di- or polycarboxylic acid or a reactive equivalent thereof to form an amide or imide compound. A particularly suitable acylating agent is a hydrocarbyl substituted succinic acid, ester, anhydride, mono-acid/mono-ester, or diacid. In some approaches, the hydrocarbyl substituted acylating agent is a hydrocarbyl substituted dicarboxylic acid or anhydride derivative thereof, a fatty acid, or mixtures thereof. The hydrocarbyl substituent may have a molecular weight of 700 or more as discussed above.

In other approaches, the hydrocarbyl substituted acylating agent may be carboxylic acid or anhydride reactant. In one approach, the hydrocarbyl substituted acylating agent may be selected from stearic acid, oleic acid, linoleic acid, linolenic acid, palmitic acid, palmitoleic acid, lauric acid, myristic acid, myristoleic acid, capric acid, caprylic acid, arachidic acid, behenic acid, erucic acid, anhydride derivatives thereof, or a combination thereof.

In one approach, the hydrocarbyl substituted acylating agent suitable for the second quaternary ammonium salt additive is a hydrocarbyl substituted dicarboxylic anhydride of Formula IX



(Formula IX)

wherein  $R_{21}$  of Formula IX is a hydrocarbyl or alkenyl group having a high molecular weight of about 300 or higher. In some aspects,  $R_{21}$  is a polyisobutylene group having a number average molecular weight from about 700 to about 5,000, about 700 to about 2,500, or about 700 to about 1,500. In other approaches, the number average molecular weight of  $R_{21}$  may range from about 700 to about 1300, as measured by GPC using polystyrene as a calibration reference. A particularly useful  $R_{21}$  has a number average molecular weight of about 1000 Daltons and comprises polyisobutylene.

In some approaches, the  $R_{21}$  of Formula IX is a hydrocarbyl moiety that may comprise one or more polymer units chosen from linear or branched alkenyl units. In some aspects, the alkenyl units may have from about 2 to about 10 carbon atoms. For example, the polyalkenyl radical may comprise one or more linear or branched polymer units formed from ethylene radicals, propylene radicals, butylene radicals, pentene radicals, hexene radicals, octene radicals and decene radicals. In some aspects, the  $R_{21}$  polyalkenyl radical may be in the form of, for example, a homopolymer, copolymer or terpolymer. In other aspects, the polyalkenyl radical is polyisobutylene. For example, the polyalkenyl radical may be a homopolymer of polyisobutylene comprising from about 5 to about 60 isobutylene groups, such as from about 15 to about 30 isobutylene groups. The polyalkenyl compounds used to form the  $R_{21}$  polyalkenyl radicals may be formed by any suitable methods, such as by conventional catalytic oligomerization of alkenes.

In some aspects, high reactivity polyisobutylenes having relatively high proportions of polymer molecules with a terminal vinylidene group may be used to form the  $R_{21}$  group. In one example, at least about 60%, such as about 70% to about 90%, of the polyisobutenes comprise terminal olefinic double bonds. In some aspects, approximately one mole of maleic anhydride may be reacted per mole of polyalkylene, such that the resulting polyalkenyl succinic anhydride has about 0.8 to about 1.5 succinic anhydride group per polyalkylene substituent. In other aspects, the molar ratio of succinic anhydride groups to polyalkylene groups may range from about 0.5 to about 3.5, such as from about 1 to about 1.3.

A suitable alkylating or quaternizing agent for the quaternary ammonium cationic salt additive is a hydrocarbyl-substituted carboxylate, such as an alkyl carboxylate or dialkyl carboxylate. In some approaches or embodiments, the quaternizing agent is an alkyl carboxylate selected from alkyl oxalate, dialkyl oxalate, alkyl salicylate, and combinations thereof. In other approaches or embodiments, the alkyl group of the alkyl carboxylate includes 1 to 6 carbon atoms, and is preferably methyl groups. Suitable alkylating or quaternizing agents for the second quaternary ammonium salt additive herein may be dimethyl oxalate or methyl salicylate.

For alkylation with an alkyl carboxylate, it may be desirable in some approaches that the corresponding acid of the carboxylate have a  $pK_a$  of less than 4.2. For example, the corresponding acid of the carboxylate may have a  $pK_a$  of less than 3.8, such as less than 3.5, with a  $pK_a$  of less than 3.1 being particularly desirable. Examples of suitable carboxylates may include, but not limited to, maleate, citrate, fumarate, phthalate, 1,2,4-benzenetricarboxylate, 1,2,4,5-benzenetetracarboxylate, nitrobenzoate, nicotinate, oxalate, aminoacetate, and salicylate. As noted above, preferred carboxylates include oxalate, salicylate, and combinations thereof.

Suitable examples of the quaternary ammonium cationic salt from the above described reactions for the quaternary ammonium cationic salt additive (iii) include, but are not limited to, compounds of the following exemplary structures:



wherein  $X$ ,  $R_{15}$ ,  $R_{16}$ ,  $R_{17}$ ,  $R_{21}$  and  $M$  as well as integers  $n$  and  $m$  are as described above.  $R_{22}$  is a C1 to C30 hydrocarbyl group. Due to the length of the hydrocarbyl chain and the presence of the bivalent moiety therein having, in some approaches, an internal oxygen or nitrogen atoms (i.e., the  $X$  moiety) discussed above, it is believed the quaternary ammonium salts as described herein include a relatively sterically available quaternary nitrogen that is more available for detergent activity than prior quaternary ammonium compounds.

In one approach or embodiment, the quaternary ammonium cationic salt has the following formula:



wherein  $R_{21}$  is a polyisobutylene group having a number average molecular weight from about 700 to about 1,500,  $X$  is O or HN,  $R_{15}$ ,  $R_{16}$ ,  $R_{17}$  independently are alkyl groups containing 1 to 4 carbons (e.g., methyl), and  $M$  is monomethyl oxalic anion or salicylic anion.

In some approaches, the diesel fuel herein may include about 1 to about 200 ppmv of this additive (iii), and in other approaches, about 5 to about 150 ppmv, and in yet other approaches, about 5 to about 100 ppmv, or in other approaches, about 20 to about 55 ppmv. In yet other approaches, the diesel fuel may include an amount of this additive ranging from at least about 1 ppmv, at least about 5 ppmv, or at least about 10 ppmv to less than about 200 ppmv, less than 150 ppmv, less than 100 ppmv, less than 60 ppmv, less than about 50 ppmv, less than about 30 ppmv, less than about 25 ppmv, less than about 20 ppmv, less than about 15 ppmv, or less than about 10 ppmv. In yet further approaches, a diesel fuel additive or concentrate may include, on an active basis, about 60 to about 80 weight percent of this compound. Amounts may be in by weight or by volume as needed for a particular application. In some approaches, the cationic quaternary ammonium salt may be combined with the alkoxylated phenol or phenol formaldehyde polymer discussed more below.

## 15

Hydrocarbyl Carbonyl Compound Reacted with Guanidines, Ureas, and Thioureas

Yet possible another additive in the blend to reduce measured DPF regeneration frequency when combusting diesel fuel is the reaction product of a hydrocarbyl carbonyl compound and an amine selected from guanidine, urea, thiourea, and combinations thereof. The hydrocarbyl carbonyl reactant compound of the present application can be any suitable compound having a hydrocarbyl moiety and a carbonyl moiety, and that is capable of bonding with the amine compound to form the additive compounds of the present application. Non-limiting examples of suitable hydrocarbyl carbonyl compounds include, but are not limited to, hydrocarbyl substituted succinic anhydrides, hydrocarbyl substituted succinic acids, and esters of hydrocarbyl substituted succinic acids.

As used herein and throughout this application, the term "hydrocarbyl group" or "hydrocarbyl" is used in its ordinary sense, which is well-known to those skilled in the art. Specifically, it refers to a group having a carbon atom directly attached to the remainder of a molecule and having a predominantly hydrocarbon character. Examples of hydrocarbyl groups include: (1) hydrocarbon substituents, that is, aliphatic (e.g., alkyl or alkenyl), alicyclic (e.g., cycloalkyl, cycloalkenyl) substituents, and aromatic-, aliphatic-, and alicyclic-substituted aromatic substituents, as well as cyclic substituents wherein the ring is completed through another portion of the molecule (e.g., two substituents together form an alicyclic radical); (2) substituted hydrocarbon substituents, that is, substituents containing non-hydrocarbon groups which, in the context of the description herein, do not alter the predominantly hydrocarbon substituent (e.g., halo (especially chloro and fluoro), hydroxy, alkoxy, mercapto, alkylmercapto, nitro, nitroso, and sulfoxyl); (3) hetero-substituents, that is, substituents which, while having a predominantly hydrocarbon character, in the context of this description, contain other than carbon in a ring or chain otherwise composed of carbon atoms. Hetero-atoms include sulfur, oxygen, nitrogen, and encompass substituents such as pyridyl, furyl, thienyl, and imidazolyl. In general, no more than two, or as a further example, no more than one, non-hydrocarbon substituent will be present for every ten carbon atoms in the hydrocarbyl group; in some embodiments, there will be no non-hydrocarbon substituent in the hydrocarbyl group.

In some aspects, the hydrocarbyl carbonyl compound can be a polyalkylene succinic anhydride reactant having the following Formula X:



(Formula C)

where  $R_{23}$  is a hydrocarbyl moiety, such as for example, a polyolefin radical having a number average molecular weight of from about 100 to about 10,000 daltons. For example, the number average molecular weight of  $R_{23}$  can range from about 1000 to about 5000 daltons, such as about 1200 to about 3000, as measured by GPC. Unless indicated otherwise, molecular weights in the present specification are number average molecular weights.

## 16

In some aspects,  $R_{23}$  can be a polyolefin radical comprising one or more polymer units chosen from linear or branched alkenyl units. In some aspects, the alkenyl units can have from about 2 to about 10 carbon atoms. For example, the polyolefin radical can comprise one or more linear or branched polymer units chosen from ethylene radicals, propylene radicals, butylene radicals, pentene radicals, hexene radicals, octene radicals and decene radicals. In some aspects,  $R_{23}$  can be a polyolefin radical in the form of, for example, a homopolymer, copolymer or terpolymer. In an aspect of the present disclosure, the  $R_{23}$  group can be a polyisobutylene radical. The polyolefin compounds used to form the  $R_{23}$  polyolefin radicals can be formed by any suitable methods, such as by conventional catalytic oligomerization of alkenes.

In an additional aspect, the hydrocarbyl moiety  $R_{23}$  can be derived from a linear alpha olefin or an acid-isomerized alpha olefin made by the oligomerization of ethylene by methods well known in the art. These hydrocarbyl moieties can range from about 8 carbon atoms to over 40 carbon atoms. For example, alkenyl moieties of this type can be derived from a linear  $C_{18}$  or a mixture of  $C_{20-24}$  alpha olefins or from acid-isomerized  $C_{16}$  alpha olefins.

In some aspects, high reactivity polyisobutenes having relatively high proportions of polymer molecules with a terminal vinylidene group can be used to form the  $R_{22}$  group. In one example, at least about 60%, such as about 70% to about 90%, of the polyisobutenes comprise terminal olefinic double bonds. There is a general trend in the industry to convert to high reactivity polyisobutenes, and well known high reactivity polyisobutenes are disclosed, for example, in U.S. Pat. No. 4,152,499, the disclosure of which is herein incorporated by reference in its entirety.

Specific examples of hydrocarbyl carbonyl compounds include such compounds as dodecenylsuccinic anhydrides,  $C_{16-18}$  alkenyl succinic anhydride, and polyisobutetyl succinic anhydride (PIBSA). In some embodiments, the PIBSA may have a polyisobutylene portion with a vinylidene content ranging from about 4% to greater than about 90%. In some embodiments, the ratio of the number of carbonyl groups to the number of hydrocarbyl moieties in the hydrocarbyl carbonyl compound can range from about 1:1 to about 6:1.

The hydrocarbyl carbonyl compounds can be made using any suitable method. Methods for forming hydrocarbyl carbonyl compounds are well known in the art. One example of a known method for forming a hydrocarbyl carbonyl compound comprises blending a polyolefin and maleic anhydride. The polyolefin and maleic anhydride reactants are heated to temperatures of, for example, about 150° C. to about 250° C., optionally, with the use of a catalyst, such as chlorine or peroxide.

Suitable amine compounds can be chosen from guanidines, ureas and thioureas with a  $C_5$  to  $C_{60}$  aliphatic carboxylic acid. For example, the amine can be a compound of the Formula XI, or salts thereof:



(Formula XI)

where  $X$  is  $\text{NR}_{25}$ ,  $\text{O}$  or  $\text{S}$ , wherein  $R_{25}$  is  $\text{H}$  or  $\text{C}_1$  to  $\text{C}_{15}$  hydrocarbyl; and  $R_{24}$  is  $\text{H}$ ,  $\text{NR}_{26}\text{R}_{27}$  or  $\text{C}_1$  to  $\text{C}_{20}$  hydrocarbyl or hydroxyl-substituted hydrocarbyl, wherein  $R_{26}$  and

R<sub>27</sub> can be the same or different and are H or C<sub>1</sub> to C<sub>20</sub> hydrocarbyl or hydroxyl-substituted hydrocarbyl.

In an embodiment of the present application, the amine can be chosen from the inorganic salts of guanidines, such as the halide, carbonate, nitrate, phosphate, and orthophosphate salts of guanidines. The term "guanidines" refers to guanidine and guanidine derivatives, such as aminoguanidine. In one approach, the guanidine suitable for the preparation of the additive compound is aminoguanidine bicarbonate. Guanidines, ureas, and thioureas used in the present application, including aminoguanidine bicarbonate, are readily obtainable from commercial sources, or can be prepared in a well-known manner.

The hydrocarbyl carbonyl and amine compounds described above can be mixed together under suitable conditions to provide the desired product compounds of the present disclosure. In one aspect of the present disclosure, the reactant compounds can be mixed together in a mole ratio of hydrocarbyl carbonyl to amine ranging from about 1:1.5 to about 1:2.5. For example, the mole ratio can range from about 1:1.8 to about 1:2.2, such as about 1:2.

Suitable reaction temperatures can range from about 1550° C. to about 200° C. at atmospheric pressure. For example, reaction temperatures can range from about 160° C. to about 190° C. Any suitable reaction pressures can be employed, such as, including subatmospheric pressures or superatmospheric pressures. However, the range of temperatures can be different from those listed where the reaction is carried out at other than atmospheric pressure. The reaction can be carried out for a period of time within the range of about 1 hour to about 8 hours, preferably, within the range of about 2 hours to about 6 hours.

It is believed that the resulting reaction product is an aminotriazole. For example, the reaction product can be a bistriazole. The five-membered ring of the triazoles is considered to be aromatic. The aminotriazoles are fairly stable to oxidizing agents and are extremely resistant to hydrolysis.

In one exemplary embodiment, the hydrocarbyl carbonyl is a polyisobutetyl succinic anhydride and the amine is aminoguanidine bicarbonate. These compounds can be reacted together at a ratio of about 1 mole of polyisobutetyl succinic anhydride to 2 moles aminoguanidine bicarbonate at a temperature of about 1600° C. It is believed, although it is not certain, that the reaction product is polybutenyl bis-3-amino-1,2,4-triazole. Such a product contains a relatively high nitrogen content, within the range of about 1.8 wt % to about 2.9 wt % nitrogen.

In some approaches, the diesel fuel herein may include, on an active basis, about 5 to about 50 ppmw of this additive (iv), and in other approaches, about 5 to about 30 ppmw, and in yet other approaches, about 10 to about 10 ppmw. In yet other approaches, the diesel fuel may include an amount of this additive, on an active basis ranging from at least about 5 ppmw, at least about 10 ppmw, or at least about 20 ppmw to less than about 30 ppmw, less than about 25 ppmw, less than about 20 ppmw, less than about 15 ppmw, or less than about 10 ppmw.

In yet further approaches, a diesel fuel additive or concentrate may include about 1 to about 15 weight percent of this compound.

#### Alkoxyated Phenol Resins

Yet possible another additive in the blend to reduce measured DPF regeneration frequency when combusting diesel fuel is an alkoxyated phenol polymer or an alkoxyated phenol formaldehyde polymer. Suitable alkoxyated phenol or phenol formaldehyde polymers may be obtained from a variety of sources and, while not wishing to be

limited by theory, are believed to include alkyl phenol alkoxylate or alkyl phenol formaldehyde alkoxylates as described below and, in some approaches, may include ethylene oxide and/or propylene oxide derived alkoxylation and, in other approaches, may have a molecular weight of about 1,000 to about 5,000 g/mol.

In one approach, suitable alkoxylated phenol polymers for the additives herein to reduce DPF regeneration frequency may have a general structure of



wherein PH is a phenyl group optionally substituted with R<sub>28</sub> groups where each R<sub>28</sub> is independently a C1 to C4 alkyl or alkoxy group; R<sub>29</sub> is a C1 to C10 linear or branched alkyl group (in some approaches, a C1 to C6 alkyl group, and in yet other approaches, a C3 to C5 alkyl group); AO is an alkylene oxide derived group, such as an ethylene oxide, a propylene oxide-derived group, or combinations thereof, that may vary along the (poly)alkyleneoxy chain. In Formula XII, n is an integer that may range from 1 to 100 effective to provide the desired relative solubility number for the polymer; m may be an integer of 1 or 2; and p is an integer of 0, 1 or 2. In some approaches, R<sub>28</sub> and/or R<sub>29</sub> is a branched alkyl group such as a secondary alkyl group selected from iso-propyl (prop-2-yl), sec-butyl (but-2-yl), iso-butyl (2-methyl-prop-1-yl) and/or tert-butyl group, or a 2-ethyl hexyl group, and the like, and combinations thereof.

In yet another approach, the alkoxyated phenol formaldehyde resins herein may include a total of about 30 to about 110 moles of alkoxylation within the fuel performance additive. In some instances, the alkoxyated phenol formaldehyde polymer may have about 25 to about 75 moles of alkoxylation provided by, in some approaches, ethylene oxide. In other instances, the alkoxyated phenol formaldehyde polymer may include about 5 to about 35 moles of alkoxylation provided by, in some approaches, both ethylene oxide and propylene oxide randomly within the alkoxylation moiety.

In some approaches, the diesel fuel herein may include, on an active basis, about 0.5 to about 50 ppmw of this additive (v), and in other approaches, about 1 to about 30 ppmw, and in yet other approaches, about 1 to about 10 ppmw. In yet other approaches, the diesel fuel may include an amount of this additive, on an active basis ranging from at least about 0.5 ppmw, at least about 1 ppmw, or at least about 2 ppmw to less than about 30 ppmw, less than about 25 ppmw, less than about 20 ppmw, less than about 15 ppmw, or less than about 10 ppmw. Amounts may be by volume or by weight as needed for a particular application.

#### Diesel Fuels

The fuels of the present application may be applicable to the operation of diesel engines. The fuels may include any and all middle distillate fuels, diesel fuels, biorenewable fuels, biodiesel fuel, fatty acid alkyl ester, and/or gas-to-liquid (GIL) fuels. "Biorenewable fuels" as used herein is understood to mean any fuel which is derived from resources other than petroleum. Such resources include, but are not limited to, corn, maize, soybeans and other crops; grasses, such as switchgrass, *miscanthus*, and hybrid grasses; algae, seaweed, vegetable oils; natural fats; and mixtures thereof. In an aspect, the biorenewable fuel can comprise monohydroxy alcohols, such as those comprising from 1 to about 5 carbon atoms. Non-limiting examples of suitable monohydroxy alcohols include methanol, ethanol, propanol, n-butanol, isobutanol, t-butyl alcohol, amyl alcohol, isoamyl alcohol, and mixtures thereof. Preferred fuels include gasoline fuels.

In some approaches, the diesel fuel herein includes less than about 20 weight percent of bio-generated diesel fuel selected from the groups renewable diesel, also known as highly paraffinic fuel, and fatty acid methyl esters and combinations thereof. In other approaches, the fuels include less than 15 weight percent, less than 10 weight percent, less than 5 weight percent, or less than 1 weight percent of biodiesel. In yet other approaches, the diesel fuel includes substantially no bio-generated diesel fuel, which is less than about 1 weight percent, less than about 0.5 weight percent, or none. Renewable diesel includes but is not limited to hydrotreated vegetable oil, gas-to-liquid fuel, biomass-to-liquid fuel and other highly paraffinic fuels. Fatty acid methyl esters include but are not limited to used cooking oil methyl esters, soybean methyl esters, palm methyl esters, rapeseed methyl ester and those manufactured from other vegetable oils. The diesel fuels herein are also low sulfur or ultra-low sulfur diesel fuels. As understood by those of skill, low sulfur fuels have less than 50 ppmw of sulfur, and ultra-low sulfur fuels have less than about 15 ppmw of sulfur.

The fuels herein are suitable for use in various internal combustion systems or engines. The systems or engines may include both stationary engines (e.g., engines used in electrical power generation installations, in pumping stations, etc.) and ambulatory engines (e.g., engines used as prime movers in automobiles, trucks, road-grading equipment, military vehicles, etc.). By combustion system or engine herein is meant, internal combustion engines, for example and not by limitation, Atkinson cycle engines, rotary engines, spray guided, wall guided, and the combined wall/spray guided direct injection engines. Also included are conventional and advanced port-fueled internal combustion engines, with and without advanced exhaust after-treatment systems capability, with and without turbochargers, with and without superchargers, with and without combined supercharger/turbocharger, with and without on-board capability to deliver additive for combustion and emissions improvements, and with and without variable valve timing. Further included are diesel HCCI engines, two-stroke engines, diesel fuel engines, stationary generators, diesel HCCI, supercharged, turbocharged, diesel direct injection engines, engines capable of variable valve timing, leanburn engines, engines capable of inactivating cylinders or any other internal combustion engine. Still further examples of combustion systems include any of the above-listed systems combined in a hybrid vehicle with an electric motor.

#### Other Additives

One or more optional compounds may be present in the additive and/or fuel compositions of the disclosed embodiments. For example, the additives and/or fuels may contain conventional quantities of cetane improvers, octane improvers, corrosion inhibitors, cold flow improvers (CFPP additive), pour point depressants, solvents, demulsifiers, lubricity additives, friction modifiers, amine stabilizers, combustion improvers, detergents, dispersants, antioxidants, heat stabilizers, conductivity improvers, metal deactivators, marker dyes, organic nitrate ignition accelerators, cycloaromatic manganese tricarbonyl compounds, carrier fluids, and the like. In some aspects, the compositions described herein may contain about 10 weight percent or less, or in other aspects, about 5 weight percent or less, based on the total weight of the additive concentrate, of one or more of the above additives. Similarly, the fuels may contain suitable amounts of conventional fuel blending components such as methanol, ethanol, dialkyl ethers, 2-ethylhexanol, and the like. In some approaches, however, the diesel fuel herein is

substantially free of any cetane improvers, which is less than 1 weight percent, less than 0.5 weight percent, or none.

In some aspects of the disclosed embodiments, organic nitrate ignition accelerators that include aliphatic or cycloaliphatic nitrates in which the aliphatic or cycloaliphatic group is saturated, and that contain up to about 12 carbons may be used. Examples of organic nitrate ignition accelerators that may be used are methyl nitrate, ethyl nitrate, propyl nitrate, isopropyl nitrate, allyl nitrate, butyl nitrate, isobutyl nitrate, sec-butyl nitrate, tert-butyl nitrate, amyl nitrate, isoamyl nitrate, 2-amyl nitrate, 3-amyl nitrate, hexyl nitrate, heptyl nitrate, 2-heptyl nitrate, octyl nitrate, isoctyl nitrate, 2-ethylhexyl nitrate, nonyl nitrate, decyl nitrate, undecyl nitrate, dodecyl nitrate, cyclopentyl nitrate, cyclohexyl nitrate, methylcyclohexyl nitrate, cyclododecyl nitrate, 2-ethoxyethyl nitrate, 2-(2-ethoxyethoxy)ethyl nitrate, tetrahydrofuranyl nitrate, and the like. Mixtures of such materials may also be used.

Examples of suitable optional metal deactivators useful in the compositions of the present application are disclosed in U.S. Pat. No. 4,482,357, the disclosure of which is herein incorporated by reference in its entirety. Such metal deactivators include, for example, salicylidene-o-aminophenol, disalicylidene ethylenediamine, disalicylidene propylenediamine, and N,N'-disalicylidene-1,2-diaminopropane.

Suitable optional cycloaromatic manganese tricarbonyl compounds which may be employed in the compositions of the present application include, for example, cyclopentadienyl manganese tricarbonyl, methylcyclopentadienyl manganese tricarbonyl, indenyl manganese tricarbonyl, and ethylcyclopentadienyl manganese tricarbonyl. Yet other examples of suitable cycloaromatic manganese tricarbonyl compounds are disclosed in U.S. Pat. Nos. 5,575,823 and 3,015,668, both of which are incorporated by reference in their entirety.

Other commercially available detergents and/or additives may be used in combination with the reaction products described herein. Such detergents include but are not limited to succinimides, Mannich base detergents, quaternary ammonium compounds, bis-aminotriazole detergents as generally described in U.S. patent application Ser. No. 13/450,638, and a reaction product of a hydrocarbyl substituted dicarboxylic acid, or anhydride and an aminoguanidine, wherein the reaction product has less than one equivalent of amino triazole group per molecule as generally described in U.S. patent application Ser. Nos. 13/240,233 and 13/454,697.

The additives of the present application, including the combination of additives as described above, and any optional additives used in formulating the fuels of this disclosure may be blended into a base fuel individually or in various sub-combinations. In some embodiments, the additive components of the present application may be blended into the fuel concurrently using an additive concentrate, as this takes advantage of the mutual compatibility and convenience afforded by the combination of ingredients when in the form of an additive concentrate. Also, use of a concentrate or as discussed herein, a diesel fuel additive, may reduce blending time and lessen the possibility of blending errors.

#### Methods of DPF Regeneration and Measuring Frequency Thereof

The methods herein include the combustion of the diesel fuel and the selected additives together with, in some approaches, an excess injection of diesel fuel to provide the regeneration of the DPF and also the measurement of the DPF regeneration frequency. The step of regenerating the

diesel particulate filter while combusting the diesel fuel (and optional excess diesel fuel) may be controlled and measured using a variety of techniques. For example and in some embodiments, a thermocouple may be used to measure an exhaust temperature. In one approach, an exhaust gas temperature of about 4800 to about 482° C. (900° F.) may be used as a separation point to differentiate between normal operation and regeneration. That is, one regeneration cycle starts when the exhaust gas temperature is about 480° to about 482° C. (900° F.) or above and ends when the exhaust gas temperature drops below about 480° to about 482° C. (9000° F.). In some embodiments, the regeneration temperatures may be briefly interrupted by idle periods where the vehicle is not able to maintain the exhaust temperature required for the exothermic reaction in a catalyst (DOC) and consequently the diesel particulate filter. The engine may pause the regeneration during such idle or low revving periods and then re-start the regeneration cycle when the exhaust temperature can be elevated again higher revving. In such instances that the pause is less than about 20 minutes (less than about 15 minutes, less than about 10 minutes, less than about 5 minutes, less than about 2 minutes, or less than about 1 minute), such pause would not entail multiple regeneration cycles and would be considered herein as one regeneration cycle.

As discussed previously, passive regeneration occurs when the engine typically is under high RPM or high load conditions such that injection of excess diesel fuel into a cylinder can react with the catalyst (DOC) causing a temperature rise across the catalyst and subsequently into the diesel particulate filter. This elevated temperature oxidizes and/or burns the soot and other debris trapped in the ceramic and/or diesel particulate filter and regenerates/cleans the diesel particulate filter. In other approaches, active regeneration may occur whereby the vehicle ECU also adjust engine parameters in addition to the excess fuel injection in order to achieve the desired temperatures. As noted above, one regeneration cycle is measured to begin when the exhaust stream exceeds about 4800 to about 482° C. (900° F.) and measured to stop when the exhaust stream falls below about 480° to about 482° C., although this threshold temperature is not meant to be limiting. In some embodiments, the regeneration is measured to begin and stop when the exhaust stream exceeds and subsequently falls below about 3250° C., about 3500° C., about 3750° C., about 400° C., about 4250° C., about 4500° C., about 4750° C., about 4800° C., about 5000° C., or about 6000° C. Regeneration temperatures may be between about 3000° C. to about 9000° C. In some embodiments, the reduction in diesel particulate filter regeneration frequency occurs immediately upon combusting the diesel fuel containing the one or more additives.

As noted above, the regeneration step may refer to an active regeneration and/or a passive regeneration. An active regeneration step is triggered when the exhaust and catalyst temperature is not high enough to light off the diesel oxidation catalyst so the engine control unit (ECU) adjusts engine parameters (injection timing, turbo geometry, etc.) to increase exhaust temperature while injecting excess fuel into the cylinder to cause an exothermic reaction which oxidizes the soot in the diesel particulate filter. A passive regeneration step can be triggered at high RPM/high load conditions where the engine exhaust temperature is already high enough to facilitate the reaction of excess fuel in the diesel oxidation catalyst and the engine control unit only needs to inject excess fuel for the regeneration to occur.

In other embodiments, the regeneration step may be initiated when extra diesel fuel is injected into the engine to

raise the temperature of the diesel particulate filter to a temperature above 300° F. For example, in some embodiments, the active regeneration occurs when the exhaust gas stream exceeds 300° C. and the reduction in total average regeneration time occurs immediately upon combusting the diesel fuel during an active regeneration cycle. In some embodiments, the total active regeneration time is measured through the vehicle On-Board Diagnostic (OBD) system by determining the mileage accumulated between a start and stop point that the OBD system identifies active regeneration is occurring. In other approaches, the regeneration occurs when the exhaust gas temperature exceeds the noted predetermined temperature as described previously. In some embodiments, the regeneration occurs via the engine management system increasing the exhaust gas temperature of the engine through injection of the diesel fuel into the exhaust gas stream or injection of the diesel fuel into the engine cylinder on an exhaust stroke of the engine cylinder.

When combusting the low or ultra-low sulfur diesel fuel and select additive blend described in any of the above paragraphs, the measured frequency of regeneration of the diesel filter when combusting diesel fuel including the one or more additives herein is lower than the measured frequency regeneration time per 1000 miles when combusting a diesel fuel in the engine without the one or more additives. In some aspects, the total regeneration frequency per 1000 miles of the diesel particulate filter using the diesel fuel comprising one or more of (i) the hydrocarbyl substituted dicarboxylic anhydride derivative, (ii) the quaternary ammonium internal salt, (iii) the quaternary ammonium cationic salt; (iii) the reaction product of the hydrocarbyl carbonyl compound and the amine compound; or (v) the alkoxyated phenol or phenol formaldehyde polymer may be reduced by about 0.2%, reduced by about 2%, reduced by about 5%, about 10%, reduced by about 15%, reduced by about 20%, reduced by about 25%, reduced by about 30%, reduced by about 35%, reduced by about 40%, reduced by about 45%, reduced by about 50%, reduced by about 55%, or reduced by about 60% relative to the active total regeneration time of the diesel particulate filter when combusting a diesel fuel in the engine without one or more of additives. More particularly, reductions in DPF regeneration frequency may be about 0.5 to about 20 percent.

#### Definitions

For purposes of this disclosure, the chemical elements are identified in accordance with the Periodic Table of the Elements, CAS version, Handbook of Chemistry and Physics, 75th Ed. Additionally, general principles of organic chemistry are described in "Organic Chemistry", Thomas Sorrell, University Science Books, Sausalito: 1999, and "March's Advanced Organic Chemistry", 5th Ed., Ed.: Smith, M. B. and March, J., John Wiley & Sons, New York: 2001, the entire contents of which are hereby incorporated by reference.

As used herein, the term "active regeneration" is when the exhaust and catalyst temperature is not high enough to light off the diesel oxidation catalyst (DOC) so the engine control unit (ECU) adjusts the engine parameters (e.g., injection timing, turbo geometry, etc.) to increase exhaust temperature while injecting excess fuel into the cylinder to cause an exothermic reaction that oxidizes the soot in the diesel particulate filter and cleans or "regenerates" it.

As used herein, the term "passive regeneration" is when the engine exhaust temperature is already high enough to facilitate the reaction of excess fuel in the diesel oxidation

catalyst and the ECU only needs to inject excess fuel for the regeneration to occur typically occurring at high RPM/high load conditions.

As used herein, the term "major amount" is understood to mean an amount greater than or equal to 50 wt. %, for example from about 80 to about 98 wt. % relative to the total weight of the composition. Moreover, as used herein, the term "minor amount" is understood to mean an amount less than 50 wt. % relative to the total weight of the composition.

As described herein, compounds may optionally be substituted with one or more substituents, such as are illustrated generally above, or as exemplified by particular classes, subclasses, and species of the disclosure.

As used herein, an "alkyl" group refers to a saturated aliphatic hydrocarbon group containing (unless otherwise noted in this disclosure) 1-12 (e.g., 1-8, 1-6, or 1-4) carbon atoms. An alkyl group can be straight or branched. Examples of alkyl groups include, but are not limited to, methyl, ethyl, propyl, isopropyl, butyl, isobutyl, sec-butyl, tert-butyl, n-pentyl, n-heptyl, or 2-ethylhexyl. An alkyl group can be substituted (i.e., optionally substituted) with one or more substituents such as halo, phospho, cycloaliphatic [e.g., cycloalkyl or cycloalkenyl], heterocycloaliphatic [e.g., heterocycloalkyl or hetero cycloalkenyl], aryl, heteroaryl, alkoxy, aroyl, heteroaroyl, acyl [e.g., (aliphatic)carbonyl, (cycloaliphatic)carbonyl, or (heterocycloaliphatic)carbonyl], nitro, cyano, amido [e.g., (cycloalkylalkyl)carbonylamino, arylcarbonylamino, aralkylcarbonylamino, (heterocyclo alkyl)carbonylamino, (heterocycloalkylalkyl)carbonylamino, heteroarylcarbonylamino, heteroaralkylcarbonylamino alkylaminocarbonyl, cycloalkylaminocarbonyl, heterocyclo alkylaminocarbonyl, arylaminocarbonyl, or heteroarylaminocarbonyl], amino [e.g., aliphaticamino, cycloaliphaticamino, or heterocycloaliphaticamino], sulfonyl [e.g., aliphatic-SO<sub>2</sub>—], sulfinyl, sulfanyl, sulfoxyl, urea, thiourea, sulfamoyl, sulfamide, oxo, carboxy, carbamoyl, cycloaliphaticoxy, heterocycloaliphaticoxy, aryloxy, heteroaryloxy, aralkyloxy, heteroarylalkyloxy, alkoxy carbonyl, alkylcarbo-nyloxy, or hydroxy. Without limitation, some examples of substituted alkyls include carboxyalkyl (such as HOOC-alkyl, alkoxy carbonylalkyl, and alkylcarbonyloxyalkyl), cyanoalkyl, hydroxyalkyl, alkoxyalkyl, acylalkyl, aralkyl, (alkoxyaryl)alkyl, (sulfonylamino)alkyl (such as (alkyl-SO<sub>2</sub>-amino)alkyl), aminoalkyl, amidoalkyl, (cycloaliphatic)alkyl, or haloalkenyl.

As used herein, an "alkenyl" group refers to an aliphatic carbon group that contains (unless otherwise noted in this disclosure) 2-8 (e.g., 2-12, 2-6, or 2-4) carbon atoms and at least one double bond. Like an alkyl group, an alkenyl group can be straight or branched. Examples of an alkenyl group include, but are not limited to allyl, isoprenyl, 2-butenyl, and 2-hexenyl. An alkenyl group can be optionally substituted with one or more substituents such as halo, phospho, cycloaliphatic [e.g., cycloalkyl or cycloalkenyl], heterocycloaliphatic [e.g., heterocycloalkyl or hetero cycloalkenyl], aryl, heteroaryl, alkoxy, aroyl, heteroaroyl, acyl [e.g., (aliphatic)carbonyl, (cycloaliphatic)carbonyl, or (heterocycloaliphatic)carbonyl], nitro, cyano, amido [e.g., (cycloalkylalkyl)carbonylamino, arylcarbonylamino, aralkylcarbonylamino, (hetero cycloalkyl) carbonylamino, (heterocyclo alkylalkyl) carbonylamino, heteroarylcarbonylamino, heteroaralkylcarbonylamino alkylaminocarbonyl, cycloalkylaminocarbonyl, hetero cyclo alkylaminocarbonyl, arylaminocarbonyl, or heteroarylaminocarbonyl], amino [e.g., aliphaticamino, cycloaliphaticamino, heterocyclo aliphaticamino, or aliphatic-sulfonylamino], sulfonyl [e.g., alkyl-SO<sub>2</sub>—, cycloaliphatic-SO<sub>2</sub>—, or aryl-SO<sub>2</sub>—], sulfinyl, sulfanyl, sulfoxyl,

urea, thiourea, sulfamoyl, sulfamide, oxo, carboxy, carbamoyl, cycloaliphaticoxy, heterocycloaliphaticoxy, aryloxy, heteroaryloxy, aralkyloxy, heteroaralkoxy, alkoxy carbonyl, alkylcarbonyloxy, or hydroxy. Without limitation, some examples of substituted alkenyls include cyanoalkenyl, alkoxyalkenyl, acylalkenyl, hydroxyalkenyl, aralkenyl, (alkoxyaryl)alkenyl, (sulfonylamino)alkenyl (such as (alkyl-SO<sub>2</sub>-amino)alkenyl), aminoalkenyl, amidoalkenyl, (cycloaliphatic)alkenyl, or haloalkenyl.

Unless used otherwise, a hydrocarbyl group refers to a group that has a carbon atom directly attached to a remainder of the molecule and each hydrocarbyl group is independently selected from hydrocarbon substituents, and substituted hydrocarbon substituents may contain one or more of halo groups, hydroxyl groups, alkoxy groups, mercapto groups, nitro groups, nitroso groups, amino groups, sulfoxyl groups, pyridyl groups, furyl groups, thienyl groups, imidazolyl groups, sulfur, oxygen and nitrogen, and wherein no more than two non-hydrocarbon substituents are present for every ten carbon atoms in the hydrocarbyl group.

As used herein, fuel-soluble generally means that the substance should be sufficiently soluble (or dissolve) at about 20° C. in the base fuel at least at the minimum concentration required for the substance to serve its intended function. Preferably, the substance will have a substantially greater solubility in the base fuel. However, the substance need not dissolve in the base fuel in all proportions.

The number average molecular weight (Mn) for any approach, aspect, embodiment or Example herein may be determined with a gel permeation chromatography (GPC) instrument obtained from Waters or the like instrument and data as processed with Waters Empower Software or the like software. The GPC instrument may be equipped with a Waters Separations Module and Waters Refractive Index detector (or the like optional equipment). The GPC operating conditions may include a guard column, 4 Agilent PLgel columns (length of 300×7.5 mm; particle size of 5μ, and pore size ranging from 100-10000 Å) with the column temperature at about 40° C. Unstabilized HPLC grade tetrahydrofuran (THF) may be used as solvent, at a flow rate of 1.0 mL/min. The GPC instrument may be calibrated with commercially available polystyrene (PS) standards having a narrow molecular weight distribution ranging from 500-380,000 g/mol. The calibration curve can be extrapolated for samples having a mass less than 500 g/mol. Samples and PS standards can be in dissolved in THE and prepared at concentration of 0.1-0.5 wt. % and used without filtration. GPC measurements are also described in U.S. Pat. No. 5,266,223, which is incorporated herein by reference. The GPC method additionally provides molecular weight distribution information; see, for example, W. W. Yau, J. J. Kirkland and D. D. Bly, "Modern Size Exclusion Liquid Chromatography", John Wiley and Sons, New York, 1979, also incorporated herein by reference.

A better understanding of the present disclosure and its many advantages may be clarified with the following examples. The following examples are illustrative and not limiting thereof in either scope or spirit. Those skilled in the art will readily understand that variations of the components, methods, steps, and devices described in these examples can be used. Unless noted otherwise or apparent from the context of discussion, all percentages, ratios, and parts noted in this disclosure are by weight.

## EXAMPLES

Experiments were performed to evaluate a measured regeneration time and/or measured regeneration frequency

## 25

of a diesel particulate filter using different additive compositions including one or more additives:

(i-1) a reaction product of a polyisobutylene (Mn 1000) substituted succinic anhydride (PIBSA) and tetraethylenepentaamine;

(i-2) another reaction product of a polyisobutylene (Mn 1000) substituted succinic anhydride (PIBSA) and tetraethylenepentaamine;

(ii) quaternary ammonium salt; and/or

(iii) a reaction product of polyisobutylene (Mn 1000) succinic acid and aminoguanidine bicarbonate.

## Example 1

A first exemplary diesel fuel additive was prepared by blending about 10 to about 50 weight percent of additives (i-1) and (iii) combined in a diesel additive package also including demulsifiers, lubricity agents, and solvents. A pre-blend of (i-1) and (iii) was about 20 to about 50 weight percent of (i-1) and about 2 to about 25 weight percent of (iii) with the remainder being solvent.

## Example 2

A second exemplary diesel fuel additive was prepared by blending about 10 to about 50 weight percent (i-1) and (iii) combined in a diesel additive package also including demulsifiers and solvents. The pre-blend of (i-1) and (iii) in the additive was as described in Example 1.

## Example 3

A third exemplary diesel fuel additive was prepared by blending about 10 to about 50 weight percent of additives (i-2) and (ii) combined in a diesel additive package also including demulsifiers, copper passivators, antifoam agents, and solvents. The combination of (i-1) and (ii) in the additive was about 2 to about 20 weight percent of (i-2) and about 10 to about 30 weight percent of (ii). This diesel additive package included 2 to about 13 weight percent of a tolyl-triazole copper passivator.

## Example 4

A fourth exemplary diesel fuel additive was prepared by blending about 10 to about 50 weight percent of additives (i-2) and (ii) combined in a diesel additive package also including demulsifiers, copper passivators, antifoam agents, and solvents. The combination of (i-1) and (ii) in the additive was about 8 to about 35 weight percent of (i-2) and about 1 to about 14 weight percent of (ii). This diesel additive package included 0.5 to about 10 weight percent of a tolyltriazole copper passivator.

## Example 5

Turning to FIG. 1, about 300 to about 500 ppmw of the diesel fuel additive of Example 4 was added to ultra-low sulfur diesel fuel (Colonial ultra-low sulfur diesel fuel having less than 15 ppm sulfur) and combusted in a 2016 Chevrolet Colorado diesel (2.8 L 14 Turbo, high pressure common rail engine). Vehicle preparation include sonically cleaning the injectors, changing the oil, and one DPF forced regeneration before each test started. The test consisted of a dirty-up phase combusting the ultra-low diesel fuel without any additive of Example 4 and then a DPF reduction phase combusting the ultra-low diesel fuel including the additive of Example 4.

## 26

Results are shown in FIG. 1 illustrating the regeneration frequency of each regeneration cycle during the appropriate phase. By measuring the amount of time spent at the initiation of the regeneration cycle, the total time of the active regeneration step can be estimated. Time spent for regeneration was determined as discussed above and when the exhaust temperature increased above about 480 to about 4800° C. As illustrated in FIG. 1, the DPF regeneration phase using the diesel fuel containing the additive of Example 4 provides an immediate reduction in regeneration frequency for the diesel particulate filter as clearly shown by the downward trend as compared to the upward trend of the frequency using the unadditized or base fuel. In this Example, regeneration numbers 1 to 42 were baseline and did not include any DPF reduction additives, and regeneration numbers 47 to the end were fuel including the DPF reduction additives herein. Regeneration frequency is the number of regenerations per 1000 miles and is determined by first calculating the number of miles between regeneration cycles, and then dividing 1000 miles by the mileage between cycles (for instance, if 500 miles passed between regenerations, then the regeneration frequency would be 1000/500 or 2 regenerations per 1000 miles.)

## Example 6

Further tests comparing the dirty-up phase with no-additive to a DPF reduction phase using the additive of Example 1, Example 2, or Example 4 at various treat rates. It is expected that the Dirty Up diesel fuel compositions will demonstrate increased regeneration frequency as compared to diesel fuels containing the one or more of the additives provided in Examples 1, 2, and 4 which are expected to demonstrate less frequent regeneration and better fuel efficiency similar to the results of Example 5.

## Example 7

Further experiments were performed to measure the number of regenerations of a vehicle's diesel particulate filter based on type of additive(s) added to a ultra-low sulfur diesel fuel (Colonial ultra-low sulfur diesel fuel having less than 15 ppm sulfur) as described in Example 5. The fuel additives evaluated for these experiments are included in Table 1 below.

TABLE 1

| Diesel Fuel Additive Types |                                                                                                                                                                                                                                            |
|----------------------------|--------------------------------------------------------------------------------------------------------------------------------------------------------------------------------------------------------------------------------------------|
| Additive                   | Type                                                                                                                                                                                                                                       |
| A                          | Hydrocarbyl substituted dicarboxylic anhydride derivative prepared by reacting a hydrocarbyl-substituted succinic acylating agent with an amine, polyamine, or alkyl amine having one or more primary, secondary, or tertiary amino groups |
| B                          | Quaternary ammonium internal salt obtained from amines or polyamines that is substantially devoid of any free anion species                                                                                                                |
| C                          | Thiazole, triazole, tolyltriazole, and/or thiadiazole                                                                                                                                                                                      |

The number of regenerations of the diesel particulate filter, as determined by the vehicle's on board computer, were counted during the testing, which was conducted for either 6000 or 3000 miles. For each test, a baseline with no additive (only the diesel fuel) was run and then a second test using the diesel fuel and the noted additive was run for the

same mileage. The number of regenerations of the diesel particulate filter during each test was counted. Results are provided below in Table 2.

TABLE 2

| Test | Length (miles) | # of DPF Regenerations | Test Results |                                                  |
|------|----------------|------------------------|--------------|--------------------------------------------------|
|      |                |                        | Additive     | Observations                                     |
| 1    | 6000           | 44                     | none         | —                                                |
| 2    | 6000           | 36                     | A + B + C    | 18% fewer regenerations than baseline test 1     |
| 3    | 6000           | 43                     | None         | —                                                |
| 4    | 6000           | 40                     | A            | Only 6% fewer regenerations than baseline test 3 |
| 5    | 3000           | 21                     | None         | —                                                |
| 6    | 3000           | 20                     | B            | Only 4% fewer regenerations than baseline test 5 |
| 7    | 3000           | 20                     | None         | —                                                |
| 8    | 3000           | 23                     | A + B        | 15% more regenerations than baseline test 7      |

As shown in Table 2 above, the combination of additives A, B, and C together in the diesel fuel has substantially fewer total regenerations over the tested mileage than additives A and B alone and even A and B combined in the diesel fuel. Notably, when just A and B are run together, the number of regenerations was substantially worse. It was unexpected that combinations of additives A, B, and C together in a diesel fuel would lead to a drop in the number of diesel particulate filter regenerations given that using A and B together was worse.

During these experiments, the pressure drop across the diesel particulate filter was also measured using the voltage output from the differential pressure sensor on the filter. The plot of the pressure for run 1 (no additive—first 6000 miles of the chart) and run 2 (A+B+C as the additive—second 6000 miles of the chart) is provided in FIG. 2. This shows that the back pressure on the filter did not change between run 1 with no additive and run 2 with the combination of all three additives. Thus, the back pressure on the diesel particulate filter is not related to the number of regenerations of the filter because the back pressure was the same between tests 1 and 2, but the number of regeneration of test 2 was 18% lower even though the filter back pressure remained constant.

#### Example 8

Another exemplary diesel fuel additive was prepared by blending about 15 to about 30 weight percent of a quaternary ammonium cationic salt (as described in U.S. Pat. No. 10,308,888, which is incorporated herein by reference) and about 0.5 to about 2 weight percent of alkoxylated phenol formaldehyde polymers in a diesel additive package also including antifoam agents and solvents.

#### Example 9

Further tests comparing the dirty-up phase with no additive to a DPF reduction phase using the additive of Table 3 below (consistent to Example 8) at various treat rates. It is expected that the Dirty Up diesel fuel compositions (having less than 15 ppm of sulfur and no additives) will demonstrate increased regeneration frequency as compared to diesel fuels containing the additives provided in Table 3 below which are expected to demonstrate less frequent regeneration and better fuel efficiency similar to the results of Example 5.

TABLE 3

| 5  | Additive | Diesel Fuel Additives                                                                                                                                                                                                         |  |
|----|----------|-------------------------------------------------------------------------------------------------------------------------------------------------------------------------------------------------------------------------------|--|
|    |          | Type                                                                                                                                                                                                                          |  |
| 10 | D        | Alkoxylated phenol or phenol-formaldehyde polymer                                                                                                                                                                             |  |
|    | E        | Quaternary ammonium cationic salt obtained from a hydrocarbyl substituted acylating agent reacted with ether amines and quaternized with dimethyl oxalate or methyl salicylate quaternizing agents (U.S. Pat. No. 10,308,888) |  |

It is anticipated that the number of regenerations of the diesel particulate filter, as determined by the vehicle's on board computer, when conducted for either 6000 will be within the ranges of Table 4 below. For each test, a baseline will be performed with no additive (only the diesel fuel) and then a second test using the diesel fuel and the noted additive of table 4 will be performed. The number of regenerations of the diesel particulate filter during each test will be counted. Treat rates will be about 1 to 10 ppmv of D and 40 to 55 ppmv of E. Expected results are provided below in Table 4.

TABLE 4

| 25 | Test Results |                |                                 |          |                                                                                      |
|----|--------------|----------------|---------------------------------|----------|--------------------------------------------------------------------------------------|
|    | Test         | Length (miles) | # of Expected DPF Regenerations | Additive | Observations                                                                         |
| 30 | 1            | 6000           | >60                             | none     | Expected number of regenerations on un-additized diesel fuel                         |
|    | 2            | 6000           | <60                             | D + E    | Expect fewer regenerations than baseline test 1 when using combinations of additives |

During these experiments, the pressure drop across the diesel particulate filter will be monitored using the voltage output from the differential pressure sensor on the filter. It is expected that the back pressure on the filter will not change between run 1 with no additive and run 2 with the combination of additives consistent to FIG. 2. Thus, without wishing to be limited by theory, it will be expected that the back pressure on the diesel particulate filter will not be related to the number of regenerations of the filter.

It is noted that, as used in this specification and the appended claims, the singular forms "a," "an," and "the," include plural referents unless expressly and unequivocally limited to one referent. Thus, for example, reference to "an antioxidant" includes two or more different antioxidants. As used herein, the term "include" and its grammatical variants are intended to be non-limiting, such that recitation of items in a list is not to the exclusion of other like items that can be substituted or added to the listed items.

For the purposes of this specification and appended claims, unless otherwise indicated, all numbers expressing quantities, percentages or proportions, and other numerical values used in the specification and claims, are to be understood as being modified in all instances by the term "about." Accordingly, unless indicated to the contrary, the numerical parameters set forth in the following specification and attached claims are approximations that can vary depending upon the desired properties sought to be obtained by the present disclosure. At the very least, and not as an attempt to limit the application of the doctrine of equivalents to the scope of the claims, each numerical parameter should

at least be construed in light of the number of reported significant digits and by applying ordinary rounding techniques.

It is to be understood that each component, compound, substituent or parameter disclosed herein is to be interpreted as being disclosed for use alone or in combination with one or more of each and every other component, compound, substituent or parameter disclosed herein.

It is further understood that each range disclosed herein is to be interpreted as a disclosure of each specific value within the disclosed range that has the same number of significant digits. Thus, for example, a range from 1 to 4 is to be interpreted as an express disclosure of the values 1, 2, 3 and 4 as well as any range of such values.

It is further understood that each lower limit of each range disclosed herein is to be interpreted as disclosed in combination with each upper limit of each range and each specific value within each range disclosed herein for the same component, compounds, substituent or parameter. Thus, this disclosure to be interpreted as a disclosure of all ranges derived by combining each lower limit of each range with each upper limit of each range or with each specific value within each range, or by combining each upper limit of each range with each specific value within each range. That is, it is also further understood that any range between the endpoint values within the broad range is also discussed herein. Thus, a range from 1 to 4 also means a range from 1 to 3, 1 to 2, 2 to 4, 2 to 3, and so forth.

Furthermore, specific amounts/values of a component, compound, substituent or parameter disclosed in the description or an example is to be interpreted as a disclosure of either a lower or an upper limit of a range and thus can be combined with any other lower or upper limit of a range or specific amount/value for the same component, compound, substituent or parameter disclosed elsewhere in the application to form a range for that component, compound, substituent or parameter.

While particular embodiments have been described, alternatives, modifications, variations, improvements, and substantial equivalents that are or can be presently unforeseen can arise to applicants or others skilled in the art. Accordingly, the appended claims as filed and as they can be amended are intended to embrace all such alternatives, modifications variations, improvements, and substantial equivalents.

What is claimed is:

1. A method of reducing measured regeneration frequency of a diesel particulate filter in a vehicle combusting diesel fuel, the method comprising:

(a) combusting a diesel fuel in a vehicle engine, wherein the vehicle includes a diesel particulate filter associated with the engine and wherein the diesel particulate filter requires regeneration thereof, the diesel fuel having less than about 50 ppm of sulfur and one or more additives selected from

a quaternary ammonium cationic salt obtained from amines or polyamines and dialkyl oxalate, alkyl salicylate, or a combination thereof; having the structure of Formula VII:



wherein each X is a bivalent moiety selected from the group consisting of —O—, —N(R<sub>20</sub>)—, —C(O)—, —C(O)O—, or —C(O)NR<sub>20</sub>; each R<sub>15</sub>, R<sub>16</sub>, and R<sub>17</sub> are independently alkyl groups containing 1 to 8 carbon atoms; R<sub>18</sub> and R<sub>19</sub> are independently selected from an

alkyl group, acyl group, or a hydrocarbyl substituted acyl group, the hydrocarbyl substituent of one or both of R<sub>18</sub> and R<sub>19</sub> having a number average molecular weight of about 700 or greater; R<sub>20</sub> is independently a hydrogen or a group selected from C<sub>1-6</sub> aliphatic, phenyl, or alkylphenyl; each m is independently an integer of 0 or 1 with at least one m being 1; each n is independently an integer of 1 to 10; and M<sup>⊖</sup> is a carboxylate;

- (b) regenerating the diesel particulate filter while combusting the diesel fuel; and
- (c) comparing the frequency of regeneration of the diesel particulate filter when combusting the diesel fuel comprising the one or more additives with the frequency of regeneration of the diesel particulate filter when combusting a diesel fuel which is devoid of the one or more additives; wherein the frequency of regenerations per 1000 miles of the diesel particulate filter when combusting the diesel fuel comprising the one or more additives is lower than a frequency of regenerations per 1000 miles of the diesel particulate filter when combusting a diesel fuel in the engine devoid of the one or more additives.

2. The method of claim 1, wherein the carboxylate of Formula VII is oxalate, salicylate, or combinations thereof.

3. The method of claim 2, wherein X of Formula VII is —O— or —NH—.

4. The method of claim 3, wherein the amine used to form the quaternary ammonium cationic salt additive has the structure of Formula VIII



wherein each X is a bivalent moiety selected from the group consisting of —O—, —N(R<sub>20</sub>)—, —C(O)—, —C(O)O—, or —C(O)NR<sub>20</sub>; each R<sub>15</sub> and R<sub>16</sub>, are independently alkyl groups containing 1 to 8 carbon atoms; each m is independently an integer of 0 or 1 with at least one m being 1; each n is independently an integer of 1 to 10.

5. The method of claim 4, wherein X is an oxygen atom or nitrogen atom.

6. The method of claim 4, wherein X is an oxygen atom.

7. The method of claim 4, wherein the quaternary ammonium cationic salt additive of Formula VII is derived from 3-(2-(dimethylamino)ethoxy)propylamine, N,N-dimethyl dipropylenetriamine, or mixtures thereof.

8. The method of claim 1, wherein R<sub>18</sub> and R<sub>19</sub> of Formula VII, together with the nitrogen atom to which they are attached, combine to form a hydrocarbyl substituted succinimide.

9. The method of claim 8, wherein the hydrocarbyl substituent has a number average molecular weight of about 700 to about 2,500.

10. The method of claim 1, wherein X is an oxygen atom and wherein R<sup>18</sup> and R<sup>19</sup> of Formula VI, together with the nitrogen atom to which they are attached, combine to form a hydrocarbyl substituted succinimide with the hydrocarbyl substituent having a number average molecular weight of about 700 to about 1,500 as measured by GPC using polystyrene as a calibration reference.

11. The method of claim 1, wherein M is derived from dimethyl oxalate, methyl salicylate, or combinations thereof.

12. The method of claim 1, further comprising the alkoxy-lated phenol polymer (v) having the general structure of Formula XII:



wherein PH is a phenyl group optionally substituted with R<sub>28</sub> groups where each R<sub>28</sub> is independently a C1 to C4 alkyl or alkoxy group; R<sub>29</sub> is a C1 to C10 linear or branched alkyl group; AO is an alkylene oxide derived group.

13. The method of claim 12, wherein n is an integer that may range from 1 to 100; m may be an integer of 1 or 2; and p is an integer of 0, 1 or 2; and wherein R<sub>28</sub> and/or R<sub>29</sub> is a branched alkyl group selected from iso-propyl (prop-2-yl), sec-butyl (but-2-yl), iso-butyl (2-methyl-prop-1-yl) and/or tert-butyl group, or a 2-ethyl hexyl group, or combinations thereof. 5

14. The method of claim 1, wherein the diesel fuel includes about 5 ppmv to about 150 ppmv of additive.

15. The method of claim 1, wherein the regeneration occurs when the engine injects excess diesel fuel into a cylinder to increase the exhaust gas temperature to exceed a predetermined temperature and reacts with a catalyst (DOC) causing an elevated temperature across the catalyst and into the diesel particulate filter. 15

16. The method of claim 15 wherein the elevated temperature oxidizes soot trapped in or on the diesel particulate filter and regenerates or cleans the filter. 20

17. The method of claim 16, wherein the regeneration is measured when the exhaust gas stream exceeds about 480° C. 25

18. The method of claim 1, wherein the regeneration frequency per 1000 miles is about 0.5 to about 20 percent lower than the regeneration frequency per 1000 miles of a diesel fuel devoid of the one or more additives.

19. The method of claim 1 wherein diesel fuel further is free of additives selected from thiazole, triazole, thiadiazole, and combinations thereof. 30

\* \* \* \* \*